

## UNITED STATES PATENT OFFICE

2,385,764

## SAP-STAIN CONTROL

Roland Smith Shumard, St. Louis, Mo., assignor  
to Monsanto Chemical Company, St. Louis,  
Mo., a corporation of Delaware

No Drawing. Application February 7, 1942.  
Serial No. 429,951

3 Claims. (Cl. 167—38.7)

The present invention relates to the protection and preservation of wood or similar cellulosic materials, particularly green wood, and particularly for protection against insects and organisms such as mold and mildew, the decay organism, *Lenzites trabea*, and sap-stain organisms, such as the chromogenic fungus, *Ceratostomella pilifera*. Specifically the invention relates to the use of quinolinols (hydroxyquinolines), particularly 8-quinolinol (8-hydroxyquinoline) and their derivatives and compositions containing quinolinols or their derivatives for said purposes.

The main objects of the invention are to provide a composition for destroying or inhibiting growth of organisms which cause deterioration of wood; which composition is relatively inexpensive to prepare; which does not cause substantial objectionable staining of the wood; which is relatively free from objectionable odors; which has exceptionally high toxic value against fungous growths and which retains its protective action over long periods of time, even when exposed to relatively intense weathering. Other objects and advantages of the invention, some of which are referred to specifically hereinafter, will be apparent to those skilled in the art.

The action of various fungi in producing stain or decay in wood and cellulosic materials has long been recognized. Among the most common offenders are chromogenic molds, the ordinary blue or sap-staining fungi, such as *Ceratostomella pilifera*, and decay organisms, such as *Lenzites trabea* and *Poria incrassata*. Molds and sap-stain organisms are exceptionally active in relatively warm climates such as exist in the southern part of the United States and are active in green wood containing sap. Sap-stain organisms do not usually produce pronounced decomposition of the wood in which they grow, but instead they degrade the wood for certain uses and thereby cause a reduction in the value of the lumber for market purposes. Wood substances, after they have become sufficiently seasoned, and so long as they remain dry, are practically immune from sap stain and general mold growth.

It has heretofore been proposed to protect green lumber during the period of seasoning, from sap-

stain organisms by dipping, spraying, or otherwise applying thereto a suitable toxic substance having the property of inhibiting or completely preventing the growth of stain organisms. Such a substance should possess a relatively large number of characteristics, some of which are more or less the antithesis of others. The following constitutes a partial list of such properties:

- (a) The material should be inexpensive.
- (b) It should not possess an objectionable odor.
- (c) It should be highly toxic both to fungi which produce stain and decay in lumber and to molds.
- (d) It should be substantially non-toxic to higher animal life.
- (e) It should not produce substantial objectionable discoloration of lumber to which it is applied.
- (f) It should be of such nature that it can be formulated into aqueous solutions for application but it should be of only slight solubility and volatility when applied to lumber.
- (g) It should be non-corrosive to metals or to wood.
- (h) It should not operate deleteriously to paints and varnishes which may be applied to the finished wood.
- (i) It should penetrate into or adhere to the wood with relative ease.
- (j) Among the materials which have heretofore been proposed for the treatment of green wood are borax, sodium carbonate and other alkalies; phenols such as cresols and wood and coal tar derivatives; ethyl mercury chloride and other mercury chloride and other mercury derivatives; chlorinated phenols and their salts, such as trichlorophenols, trichlorocresols, tetrachlorophenols, pentachlorophenol and chlorinated phenyl-phenols (for example, 2-chloro-ortho-phenyl-phenol, i. e., 2-hydroxy-3-chloro-diphenyl or 2-chloro-6-phenyl-phenol) and their sodium salts. The chlorinated phenols have been eminently satisfactory for this use. In general, mercury derivatives are relatively ineffective against molds. The alkalies are unsatisfactory because of their relative ineffectiveness against sap-stain and mold organisms, the relatively high concen-

tration which must be used, and their effect upon wood when used at such high concentrations.

I have discovered that quinolinols (hydroxy-quinolines), particularly 8-quinolinol (8-hydroxyquinoline), either in the free form or in the form of metal salts or salts with acids, but preferably in the form of their sodium or other alkali-metal salts, are especially effective agents for the treatment of lumber to protect it from or prevent the attack of insects and growth of molds and other organisms such as the decay organism, *Lenzites trabea*, and the blue-stain organisms *Ceratostomella pilifera*. The alkali-metal salts of 8-quinolinol, such as sodium 8-quinolinolate, and the acid salts of 8-quinolinol, such as the hydrochloride or sulfate (the latter is known as quinosol, Cryptonol, Sunoxol, and Superol) are soluble in water and when applied to green wood or lumber, in the form of an aqueous solution containing 0.5% or more of the salt, provide a treatment comparable to that obtained with a 1% aqueous solution of sodium pentachlorophenate. When used in concentrations of substantially less than 0.5%, for example, about 0.25%, the growth of sap-stain organisms is prevented but the growth of certain molds persists although at a somewhat retarded rate.

I have also discovered that in admixture with alkalies such as borax the toxicity of the alkali-metal salts of the quinolinols is not substantially affected, that is, it is neither substantially reduced, nor is it definitely enhanced. However, in admixture with toxic chlorinated phenols, such as sodium pentachlorophenate, the toxicities of both the sodium 8-quinolinolate and the sodium pentachlorophenate are enhanced, that is, the two toxics appear to mutually activate each other since the toxicity of the mixture is greater than is attributable to the sum of the individual toxicities of its components. In three component mixtures containing sodium 8-quinolinolate, borax and sodium pentachlorophenate, the borax produces a slight reduction in the effectiveness that would be expected from a mixture of sodium 8-quinolinolate and sodium pentachlorophenate without borax.

As examples of the advantages to be obtained by the use of the quinolinols and their salts and compositions containing quinolinols or their salts for the protection of wood the following comparative results are typical.

Discs of green fast-growing southern yellow pine, having a diameter of about 2 1/4 inches and a thickness of about 1/2 inch, were used. These discs of wood were dipped in aqueous solutions of varying concentrations of the toxics and were then allowed to drain. Four discs were treated at each concentration. The treated discs were then sprayed with an aqueous suspension of a culture of the stain organism, *Ceratostomella pilifera*. The thus inoculated discs were placed in Mason jars, four to a jar. The four discs that were placed in each jar were those which had been treated with the same concentration of the same toxic chemical and they were separated from each other by pieces of applicator sticks or other suitable wood separators, thus assuring a complete circulation of air over all the wood surfaces. The jars were closed with a metal screw cap through which a vent about 1 inch in diameter had been punched. This vent was plugged with cotton to allow the vapors from the wood to escape and to permit slow evaporation of moisture. The jars were then incubated at a standard temperature (26° C. in these results) in a

room with a controlled humidity (65% R. H.) for a definite period (7 days) and the growths appearing thereon were observed.

The discs in most cases were treated with aqueous solutions containing 0.25, 0.5, 1.0 and 2.0 parts by weight of the toxic chemical or composition per 100 parts of water. The following solutions were used:

1. Sodium benzylphenate. The solutions were prepared from a technical mixture of ortho and para-benzylphenols, to which sufficient sodium hydroxide had been added to provide clear solutions. The amount of sodium hydroxide added was somewhat greater than the stoichiometrically required for the conversion of the phenol to the salt.

2. Sodium 2-chlorobenzylphenate. These solutions were prepared from a benzylated 2-chlorophenol and sufficient sodium hydroxide was added to effect solution.

3. Sodium trichlorocresolate. These solutions were prepared from a trichlorocresol mixture obtained by the alkaline hydrolysis of 2, 3, 4, 6-tetrachlorotoluene. Sufficient sodium hydroxide was added to convert the phenol to the sodium salt and to dissolve the phenol with the formation of clear solutions.

4. Sodium pentachlorophenate. These solutions were prepared from a commercial sodium pentachlorophenate containing a slight excess of alkali.

5. Sodium quinolinolate. These solutions were prepared from 8-quinolinol (8-hydroxyquinoline) to which was added a slight excess of sodium hydroxide over that stoichiometrically required to effect conversion of the quinolinol to sodium salt to produce a clear solution.

6. Quinosol. The same 8-quinolinol as in 5 was used. Sufficient sulfuric acid was added to convert the quinolinol to the sulfate (quinosol).

7. Sodium pentachlorophenate 50%—borax 50% mixture. The solutions were prepared from a mixture of equal parts by weight of sodium pentachlorophenate and borax ( $Na_2B_4O_7 \cdot 10H_2O$ ).

8. Sodium 8-quinolinolate 50%—borax 50% mixture. The solutions were prepared from materials hereinabove described so as to contain equal parts by weight of sodium 8-quinolinolate and borax.

9. Sodium 8-quinolinolate 50%—sodium pentachlorophenate 50% mixtures. The solutions were prepared from the materials hereinabove described so as to contain equal parts by weight of sodium 8-quinolinolate and sodium pentachlorophenate.

10. Sodium 8-quinolinolate 33 1/3%—sodium pentachlorophenate 33 1/3%—borax 33 1/3% mixture. The solutions were prepared from the materials hereinabove described so as to contain equal parity by weight of sodium 8-quinolinolate, sodium pentachlorophenate and borax.

The results after a period of incubation of 7 days at 26° C. of the above solutions at concentrations corresponding to 0.25%, 0.5%, 1% and 2% of the toxic or mixture of toxics were as follows. In all these results the molds referred to are those naturally occurring with and contaminating the wood. Experience with these discs has shown a relatively uniform contamination and it is therefore not necessary to artificially inoculate the samples with mold.

The results were tabulated as in Table I following. The "per cent area stain" is the average estimated stained area of the cross section of the four discs (eight areas) in each treatment.

Table I.—Stain and mold control with various treatments

| Composition                        | Concentration of treating solution |        |            |       |            |       |            |      |
|------------------------------------|------------------------------------|--------|------------|-------|------------|-------|------------|------|
|                                    | 0.25%                              |        | 0.5%       |       | 1%         |       | 2%         |      |
|                                    | Area stain                         | Mold   | Area stain | Mold  | Area stain | Mold  | Area stain | Mold |
| 1. Sodium benzylphenate            | Percent                            |        | Percent    | No.   | Percent    | No.   | Percent    | No.  |
| 2. Sodium 2-chlorobenzylphenate    |                                    |        | 57         | 31    | 7          | 40    | Do.        |      |
| 3. Sodium trichlorocresolate       |                                    |        | 94         | 75    | do.        | do.   | do.        | Do.  |
| 4. Sodium pentachlorophenate       |                                    |        | 47         | 0.8   | do.        | do.   | do.        | Do.  |
| 5. Sodium 8-quinolinolate          | 88                                 | No.    | 20         | 8.6   | do.        | do.   | do.        | Do.  |
| 6. Quinosol                        | 0                                  | Heavy  | 0          | 0     | do.        | do.   | do.        | Do.  |
| 7. Sodium pentachlorophenate 50%   | 0                                  | do.    | 0          | Heavy | 0          | Light | 0          | Do.  |
| 8. Borax 50%                       | 92                                 | No.    | 20         | No.   | 8          | No.   | do.        |      |
| 9. Sodium 8-quinolinolate 50%      | 0                                  | Heavy  | 0          | Heavy | 0          | do.   | do.        |      |
| 10. Sodium pentachlorophenate 50%  | 0                                  | No.    | 0          | No.   | 0          | do.   | do.        |      |
| 11. Sodium 8-quinolinolate 33 1/3% | 7.5                                | Medium | 0          | Light | 0          | Light | do.        |      |
| 12. Borax 33 1/3%                  |                                    |        |            |       |            |       |            |      |

<sup>1</sup> Red mold stain characteristic of borax treatments found at all concentrations.

In Table II the results from Table I are arranged to show the minimum concentrations of treating solutions of the various compositions which are required to provide control of stain growth and superficial mold growth. From Table II it will be apparent that all compositions containing quinolinol derivatives (5, 6, 8, 9, 10) are as effective in controlling stain as sodium pentachlorophenate alone or mixed with an equal weight of borax (4 and 7) and that the best compositions are those in which the quinolinolate is mixed with a chlorinated phenol (9). It is also to be observed that at equal concentrations the quinolinolate is more effective for stain control than sodium pentachlorophenate and that sodium pentachlorophenate is more effective for mold control than the quinolinolate (compare 4 and 5), but that a lesser quantity of a mixture of the two (see 9) can be used to provide complete control against stain and mold than either alone. It must be appreciated that the foregoing values in Table II apply only under the conditions described previously, that is, when both types of organisms are present.

Table II.—Minimum concentration of treating solution required to provide control

| Composition                                                        | Stain growth | Superficial mold growth |
|--------------------------------------------------------------------|--------------|-------------------------|
| 1. Sodium benzylphenate                                            | Per cent     | Per cent                |
| 2. Sodium 2-chlorobenzylphenate                                    | 2.0          | 0.5                     |
| 3. Sodium trichlorocresolate                                       | 1.0          | 0.5                     |
| 4. Sodium pentachlorophenate                                       | 2.0          | 0.25                    |
| 5. Sodium 8-quinolinolate                                          | 0.25         | 1.0                     |
| 6. Quinosol                                                        | 0.25         | 2.0                     |
| 7. Sodium pentachlorophenate 50%                                   | 2.0          | 0.25                    |
| 8. Borax (Na <sub>2</sub> BO <sub>3</sub> ·10H <sub>2</sub> O) 50% | 0.25         | 1.0                     |
| 9. Sodium 8-quinolinolate 50%                                      | 0.25         | 0.25                    |
| 10. Sodium pentachlorophenate 33 1/3%                              | 0.5          | 2.0                     |
| 11. Sodium 8-quinolinolate 33 1/3%                                 |              |                         |

In using the invention the wood or green lumber may be treated by any of the conventional methods for application of sap-stain chemicals. Thus, the compositions of the present invention may be applied in the form of solutions either by spraying, brushing, dipping or pressure impregnation. The quinolinol may be precipitated on the wood in the free form or in the form of

salts of heavy metals, if desired, by a second treatment with a solution of a salt of a heavy metal. The concentration of the solutions to be used will be dependent to a great extent upon the degree of control desired and the toxicity of the composition used, but will be in general be from about 0.25% to 2.0% or higher. In the case of a composition such as 9 hereinabove, a concentration of 0.25% to 0.5% is generally adequate to provide a greater degree of control than is generally necessary in the field.

The compositions for the treatment of wood to prevent sap-stain and mold growth contemplated by the present invention are those comprising a quinolinol or a metal or acid salt thereof, particularly 8-quinolinol and its sodium salt. Preferred compositions of the invention are those which comprise the quinolinol or alkali-metal salt thereof, particularly sodium 8-quinolinolate, in admixture with other toxic chemicals such as chlorinated phenols or salts thereof, for example, sodium trichlorophenates, sodium tetrachlorophenates, sodium pentachlorophenate, sodium trichlorocresolates, sodium tetrachlorocresols, and other sodium salts of chlorinated cresols and higher alkylated phenols, sodium, 2-chloro-6-phenylphenate and similar sodium salts of chlorinated phenylphenols. The compositions of the present invention may also include adjuvants such as wetting agents, for example, alkylated aromatic sulfonic acid salts such as sodium dodecylbenzenesulfonate, sodium butyldiphenylsulfonate, and the like, and other conventional ingredients.

My invention is directed to the use of quinolinols, either in the free form or in the form of metal or acid salts. The invention is directed specifically to the preferred use of 8-quinolinol derivatives, particularly the sodium salt and the sulfate (quinosol), but other isomers such as alpha- or 2-hydroxyquinoline (2-quinolinol or carbostyryl) beta- or 3-hydroxyquinoline (3-quinolinol), gamma- or 4-hydroxyquinoline (4-quinolinol or kyanurin), ana- or 5-hydroxyquinoline (5-quinolinol), para- or 6-hydroxyquinoline (6-quinolinol) and meta- or 7-hydroxyquinoline (7-quinolinol), chlorinated quinolinols and alkylated quinolinols, such as 5-chloro-8-quinolinol, 5,7-dichloro-8-quinolinol, 5-methyl-8-quinolinol, 6-methyl-8-quinolinol, and 7-chloro-5-propylquinolinol, and their acid and metal salts may be

wood. The sodium salt is formed by the addition of sodium hydroxide or sodium carbonate to the quinolinol, whereas the acid salts are formed by adding an acid, for example, hydrochloric acid or sulfuric acid, to the quinolinol. For use in the free form the invention contemplates the use of alcohol or other suitable solvents for the preparation of suitable dipping solutions. A suitable dipping solution of 8-quinolinol, for example, can be prepared by using a mixture of water containing a small proportion of ethyl alcohol.

Inasmuch as the foregoing specification comprises preferred embodiments of the invention, it is to be understood that the invention is not limited thereto and that variations and modifications may be made therein to adapt the invention to specific uses without departing substantially from the appended claims.

I claim:

1. The method of treating green wood to prevent the growth of molds and sap-staining fungi thereon, which comprises applying to the wood a solution of a mixture containing as its active constituents sodium 8-quinolinolate and sodium pentachlorophenate.
2. A green-wood mold and sap-stain control agent which contains as its active constituent a mixture of sodium 8-quinolinolate and sodium pentachlorophenate.
3. The method of treating green wood to prevent the growth of molds and sap-staining fungi thereon, which comprises applying to the wood a solution of a preservative consisting of sodium 8-quinolinolate and sodium pentachlorophenate.

ROLAND S. SHUMARD.

CERTIFICATE OF CORRECTION.

Patent No. 2,385,764.

September 25, 1945.

ROLAND SMITH SHUMARD.

It is hereby certified that error appears in the printed specification of the above numbered patent requiring correction as follows: Page 1, second column, lines 34 and 35, strike out the words "and other mercury chloride"; page 2, second column, line 14, for "than the" read --than that--; and that the said Letters Patent should be read with this correction therein that the same may conform to the record of the case in the Patent Office.

Signed and sealed this 1st day of January, A. D. 1946.

Leslie Frazer

(Seal)

First Assistant Commissioner of Patents.

wood. The sodium salt is formed by the addition of sodium hydroxide or sodium carbonate to the quinolinol, whereas the acid salts are formed by adding an acid, for example, hydrochloric acid or sulfuric acid, to the quinolinol. For use in the free form the invention contemplates the use of alcohol or other suitable solvents for the preparation of suitable dipping solutions. A suitable dipping solution of 8-quinolinol, for example, can be prepared by using a mixture of water containing a small proportion of ethyl alcohol.

Inasmuch as the foregoing specification comprises preferred embodiments of the invention, it is to be understood that the invention is not limited thereto and that variations and modifications may be made therein to adapt the invention to specific uses without departing substantially from the appended claims.

I claim:

1. The method of treating green wood to prevent the growth of molds and sap-staining fungi thereon, which comprises applying to the wood a solution of a mixture containing as its active constituents sodium 8-quinolinolate and sodium pentachlorophenate.
2. A green-wood mold and sap-stain control agent which contains as its active constituent a mixture of sodium 8-quinolinolate and sodium pentachlorophenate.
3. The method of treating green wood to prevent the growth of molds and sap-staining fungi thereon, which comprises applying to the wood a solution of a preservative consisting of sodium 8-quinolinolate and sodium pentachlorophenate.

ROLAND S. SHUMARD.

CERTIFICATE OF CORRECTION.

Patent No. 2,385,764.

September 25, 1945.

ROLAND SMITH SHUMARD.

It is hereby certified that error appears in the printed specification of the above numbered patent requiring correction as follows: Page 1, second column, lines 34 and 35, strike out the words "and other mercury chloride"; page 2, second column, line 14, for "than the" read --than that--; and that the said Letters Patent should be read with this correction therein that the same may conform to the record of the case in the Patent Office.

Signed and sealed this 1st day of January, A. D. 1946.

Leslie Frazer

(Seal)

First Assistant Commissioner of Patents.